

## UNITED STATES PATENT OFFICE

2,589,979

## SOLVENTS FOR GASOLINE INHIBITORS

Barney R. Strickland, Westfield, N. J., assignor to  
Standard Oil Development Company, a corpora-  
tion of Delaware

No Drawing. Application September 1, 1949,  
Serial No. 113,663

2 Claims. (Cl. 44—63)

1

This invention relates to the use of improved solvents for use with gasoline inhibitors. In accordance with the present invention, toluene or dioxan (diethylene dioxide) also known as paradioxan is employed to dissolve the inhibitors which are conventionally added to gasolines. This application constitutes a continuation in part of U. S. No. 790,223, filed December 6, 1947 now abandoned, which discloses the subject matter of this application.

In order to prevent the oxidation of potential gum forming substances in gasolines, and in order to prevent discoloration of the gasoline, both of which may occur, it is conventional practice to add various inhibitors to the gasoline. These inhibitors are of various types, for example, aminophenols, phenylenediamines, alpha-naphthol, trialkylphenols, and straight chain alkyl phenols. In general these inhibitors are somewhat unstable being subject to decomposition over a period of time, chiefly due to their reaction with air or oxygen. In particular, the aminophenols and the phenylenediamines are subject to degradation by oxidation. It is a particular object of this invention to minimize the degradation of these gasoline inhibitors by minimizing their tendency to react with oxygen.

It is essential that an inhibitor used with gasoline be reasonably soluble in the gasoline. This is a particularly stringent requirement in view of the present use of gasolines at extremely high altitudes and the consequently low temperatures. Consequently, it is general practice to dissolve the inhibitors in a suitable solvent prior to addition to the gasoline so as to improve the solubility of the inhibitors in the gasoline. At the present time alcohols are generally employed as the solvent, being soluble in gasolines, and being a good solvent for the inhibitors generally used. It is a further object of this invention that improved solvent action be obtained by the use of toluene or dioxan in place of the alcohols conventionally used. In view of the present wide commercial use of alcohol as the solvent for the inhibitors, this disclosure will be especially directed to show the improvement of the present solvents over alcohol.

To determine the relative solubility of inhibitors in alcohol and in the solvents employed in this invention, a typical inhibitor 2,6-di-tertiary-butyl-4-methylphenol was added to different alcohols and to toluene at 75° F. It was found that less than 20 wet. percent of the inhibitor could be dissolved in isopropyl alcohol, that 21% of the inhibitor could be dissolved in normal butyl al-

cohol, that 25% of the inhibitor could be dissolved in ethyl alcohol, and that 41% of the inhibitor could be dissolved in toluene. Further data obtained indicated that substantially 35% by weight of the inhibitor named could be dissolved in toluene without danger of crystallizing out at 0° F.

In addition to the high solvent power of toluene this solvent is advantageous in that it is relatively inexpensive and has a very high motor fuel blending value.

A still further advantage of toluene is that it is in some way effective in minimizing the air oxidation of solutions of the inhibitors. This is indicated by the following table:

Table I

| Sample                                                         | Time required for Indicated Oxygen Pressure Drop at— |        |         |        |
|----------------------------------------------------------------|------------------------------------------------------|--------|---------|--------|
|                                                                | 150° F.                                              |        | 212° F. |        |
|                                                                | 5 lb.                                                | 10 lb. | 5 lb.   | 10 lb. |
| 25% Solution of 2,6-di-t-butyl-4-methylphenol in Ethyl Alcohol | 240                                                  | 345    | 90      | 115    |
| Same as above except in toluene                                | 1,440+                                               | 1,440+ | 840     | 1,320  |

The data were obtained by containing the inhibitor and solvent in an A. S. T. M. breakdown bomb. The solutions were subjected in the bomb to 100 lb. oxygen pressure and to temperatures of 150° F. and 212° F. The time required for the pressure in the bomb to drop 5 lbs., and 10 lbs., was recorded. This time represents the time required for sufficient oxygen to react with the solutions to create the indicated pressure drop. It will be noted that the solution of the inhibitor in ethyl alcohol was subject to comparatively rapid oxidation, the oxygen pressure in the bomb dropping 5 lbs. in 240 minutes at 150° F. When the inhibitor was dissolved in toluene, however, more than 1400 minutes were required to obtain the same drop in oxygen pressure. At 212° F. the corresponding times for 5 lbs. pressure drop were 90 minutes with ethyl alcohol and 840 minutes for toluene. These data clearly indicates that the toluene when used as the solvent has a profound effect on the reactivity of the inhibitor with air. Further experiments showed that neither the alcohol or toluene alone reacted with oxygen under the test conditions.

Further experiments were conducted with other inhibitors under different test conditions. An inhibitor consisting of N,N'-di-sec-butyl-p-

phenylenediamine was dissolved in the particular solvent to be tested in a concentration of 15 grams per 100 ml. of solution. The solution of the inhibitor was then introduced into a closed system, comprising a packed tower maintained at room temperature and atmospheric air pressure, wherein it was circulated countercurrently to a stream of air. The results obtained are indicated in Table II below:

Table II

| Solvent                                   | M1. Oxygen Absorbed by 13.5 g. of N,N'-di-sec-butyl-p-phenylenediamine after— |          |          |          |          |
|-------------------------------------------|-------------------------------------------------------------------------------|----------|----------|----------|----------|
|                                           | 50' Hrs.                                                                      | 100 Hrs. | 150 Hrs. | 200 Hrs. | 250 Hrs. |
| 1. Ethyl alcohol alone.....               | 1,100                                                                         | 2,200    | 2,750    | 2,900    | 2,900    |
| 2. Toluene alone.....                     | None                                                                          | 80       | 120      | 120      | —        |
| 3. 9 Parts toluene, 1 Part ethyl alcohol. | None                                                                          | 200      | 700      | 1,300    | 1,700    |

The data showing the milliliters of oxygen absorbed by the solution were obtained by analytical methods to determine the oxygen absorption. It will be noted that the inhibitor dissolved in ethyl alcohol was extremely reactive with oxygen, absorbing 2900 ml. of oxygen in 200 hours, under the test conditions. The inhibitor dissolved in toluene, however, was comparatively unreactive with oxygen only absorbing 120 ml. after 200 hours. Considerable improvement in oxygen reactivity was notable in the case where 9 parts of toluene were used with one part of ethyl alcohol. In the first case, where the inhibitor was dissolved in ethyl alcohol, degradation was so extensive that the inhibitor became very dark and tarry and completely lost its inhibiting potency. On the other hand, the inhibitor dissolved in toluene darkened only slightly and did not materially lose its inhibiting potency. The inhibitor oxidized in toluene solution was found by analysis to contain 95% active inhibitor.

Further tests were made on a variety of inhibitors in different solvents employing A. S. T. M. breakdown bombs at a temperature of 150° F. and 30 lbs. per square inch gauge oxygen pressure. The results obtained are indicated in Table III:

Table III

| Sample                                                     | Time, Minutes, for Oxygen Pressure Drop— |         |
|------------------------------------------------------------|------------------------------------------|---------|
|                                                            | 5 lbs.                                   | 10 lbs. |
| N,N'-di-sec-butyl-p-phenylenediamine alone—no solvent..... | 270                                      | 510     |
| N,N'-di-sec-butyl-p-phenylenediamine in:                   |                                          |         |
| Methyl alcohol.....                                        | 40                                       | 55      |
| Ethyl alcohol.....                                         | 55                                       | 90      |
| Methyl propyl ketone.....                                  | 120                                      | 175     |
| Benzene.....                                               | 190                                      | 265     |
| Toluene + ethyl alcohol (90:10).....                       | 130                                      | 190     |
| Xylene.....                                                | 250                                      | 355     |
| Isooctane.....                                             | 325                                      | 525     |
| Cyclohexane.....                                           | 405                                      | 635     |
| Diisobutylene.....                                         | 280                                      | 475     |
| Dioxan.....                                                | 730                                      | 985     |
| n-butyl-p-aminophenol in:                                  |                                          |         |
| Methyl alcohol.....                                        | 25                                       | 45      |
| Isopropyl alcohol.....                                     | 65                                       | 110     |
| Methyl propyl ketone.....                                  | 55                                       | 80      |
| Dioxan.....                                                | 120                                      | 195     |

In each case 7.5 g. of inhibitor were used plus enough solvent to make 50 ml. of solution. It will be noted from the data of Table III that the inhibitors employed were markedly less reactive

with oxygen when dissolved in dioxan than in any of the other solvents employed. Thus for example in 55 minutes the oxygen bomb pressure has dropped 5 lbs. when N,N'-di-sec-butyl-p-phenylenediamine was dissolved in ethyl alcohol, while 730 minutes were required to obtain this same pressure drop when the inhibitor was dissolved in dioxan. The reactivity of the second inhibitor tested, normal butyl-p-aminophenol was similarly improved as indicated by the data for solutions in alcohol and dioxan.

To further indicate the unexpected advantages of employing toluene and dioxan as the solvents for inhibitors, N,N'-di-sec-butyl-phenylenediamine was dissolved in various solvents in a concentration of 15 grams per 100 ml. of solution and was allowed to stand at room temperature in closed bottles containing an oxygen atmosphere for a period of two days. Results of this test are given in Table IV:

Table IV

| Solvent             | Appearance— |              | Percentage of Inhibitor Potency Lost After 2 Days |
|---------------------|-------------|--------------|---------------------------------------------------|
|                     | Initially   | After 2 Days |                                                   |
| Methyl alcohol..... | Clear.....  | Dark.....    | 77                                                |
| Ethyl alcohol.....  | do.....     | do.....      | 63                                                |
| Toluene.....        | do.....     | Clear.....   | 6                                                 |
| Dioxan.....         | do.....     | do.....      | 3                                                 |

It will be noted from these data that after two days the inhibitor dissolved in either methyl alcohol or ethyl alcohol had deteriorated sufficiently so that the solution was very dark and the loss of inhibitor potency was respectively, 77% and 63%. When the inhibitor was dissolved in toluene or dioxan, however, the solution was still clear after two days and only 6% and 3%, respectively, loss of inhibitor potency occurred.

Another test was made in regard to the effect of these solvents on the potency of an inhibitor dissolved in diisobutylene. This would effectively correspond to dissolving the inhibitor in an olefinic gasoline. The inhibitor employed was N,N'-di-sec-butyl-p-phenylenediamine. Standard solutions of this inhibitor in different solvents were prepared at a concentration of 2.4 mg. of inhibitor per ml. of solution. These solutions were then added to diisobutylene to provide a concentration of 0.5 and 1 lb. of inhibitor per 5000 gallons of diisobutylene. The inhibited diisobutylene was then subjected to a standard A. S. T. M. breakdown test in which the solution tested was placed in an A. S. T. M. bomb at 212° F. under 100 lbs. per square inch oxygen pressure. The number of minutes were determined for the bomb to reach a condition at which the pressure drop in the bomb was equal to 2 lbs./sq. in. per 15 minutes. The results of this test are given in Table V:

Table V

| lbs. of N,N'-di-sec-butyl-p-phenylenediamine/5000 gallons Diisobutylene | Breakdown Time (Minutes) |
|-------------------------------------------------------------------------|--------------------------|
| Uninhibited Diisobutylene.....                                          | 85                       |
| 5 lbs dissolved in Methyl Alcohol.....                                  | 980                      |
| 1.0 lbs. dissolved in Methyl Alcohol.....                               | 1,360                    |
| 1.0 lbs. dissolved in Ethyl Alcohol.....                                | 1,120                    |
| 1.0 lbs. dissolved in Ethyl Alcohol.....                                | 1,440+                   |
| 1.0 lbs. dissolved in Toluene.....                                      | 1,440+                   |
| 1.0 lbs. dissolved in Toluene.....                                      | 1,440+                   |
| 1.0 lbs. dissolved in Dioxan.....                                       | 1,440+                   |
| 1.0 lbs. dissolved in Dioxan.....                                       | 1,440+                   |

It will be noted from this data that uninhibited diisobutylene is readily oxidized, giving a breakdown time of only 85 minutes. The oxidation is inhibited to some extent when the inhibitor is added in solution with either methyl or ethyl alcohol. However when the inhibitor is added in solution with either toluene or dioxan considerably greater inhibiting potency may be appreciated. Thus only .5 lbs. of the inhibitor per 5000 gallons of diisobutylene, when initially dissolved in toluene or dioxan, is considerably more effective than either 0.5 lbs. of the inhibitor dissolved in methyl or ethyl alcohol or even 1 lb. dissolved in methyl alcohol. Similarly this is as effective as 1 lb. of the inhibitor dissolved in ethyl alcohol. It will thus be seen that use of toluene or dioxan as the solvent for the inhibitor results in inhibiting action of improved potency.

From the data presented in this disclosure it appears that inhibitors dissolved in alcohol are extremely reactive with oxygen, resulting in discoloration of the inhibitor and loss of inhibiting potency over a period of time. When these inhibitors, however, are dissolved in dioxan or toluene they are considerably less reactive with oxygen and undergo no substantial change in color or loss in inhibiting potency. This invention, therefore, comprises employing toluene or dioxan as the solvent for the inhibitor used with gasolines. In accordance with this invention it is preferred that 25-100 weight per cent of inhibitor based on the solvent be dissolved in the solvent the inhibitor concentrates thus consist of compositions containing about 20 to 50% of inhibitor based on the total composition. The solution of the inhibitor in the solvent may then

be added to the gasoline in any desired proportions. Generally sufficient inhibitor solution is used in a gasoline to supply about 0.1-4 lbs. per 5000 gallons of inhibitor. Commonly the amount used provides about 0.5-1.0 lb. of inhibitor per 5000 gallons of fuel.

Having now described this invention, what is claimed is:

1. A composition comprising a motor gasoline, 10 a N-N'-di-secondary-butyl p-phenylenediamine and para-dioxan, said N-N'-di-secondary-butyl p-phenylenediamine being present in proportions of about 0.1 to 4 pounds per 5000 gallons, and said para-dioxan being present in proportions of 15 about 1 to 4 times the amount of N-N'-di-secondary-butyl p-phenylenediamine.
2. A motor fuel inhibitor concentrate substantially stable to oxygen containing gases which consists of para-dioxan containing about 20 to 20 50% of N-N'-di-secondary-butyl p-phenylenediamine.

BARNEY R. STRICKLAND.

#### REFERENCES CITED

25 The following references are of record in the file of this patent:

#### UNITED STATES PATENTS

| Number       | Name          | Date          |
|--------------|---------------|---------------|
| 30 2,380,420 | Emerson ----- | July 31, 1945 |
| 2,443,569    | Ruggles ----- | June 15, 1948 |

#### OTHER REFERENCES

35 Fieser and Fieser, Organic Chemistry, D. C. Heath & Co., Boston, Mass. (1944) pg. 126.